

# United States Patent Office

2,866,729

Patented Dec. 30, 1958

1

2,866,729

## QUENCHING OIL COMPOSITIONS

Carl Frederick Zimpel, East Alton, Ill., assignor to Shell Development Company, New York, N. Y., a corporation of Delaware

No Drawing. Application July 27, 1956  
Serial No. 600,390

10 Claims. (Cl. 148—29)

This invention relates to improved quenching oil compositions for use in the metallurgical industries and to the method of quenching metals therewith:

In the process of hardening metals such as steels, it is common practice to use as the quenching medium water, oil or compressed air, according to the type of steel. Recently salts or aqueous solutions of salts have also been used for this purpose but these have the disadvantage that they solidify or deposit solids on cooling to room temperature. Fatty oils, especially rapeseed oil are used as quenching oil, but these have been gradually superseded by mineral quenching oils. It has also been proposed to harden and temper steels using baths containing naphthalene mono- or di-sulphonic acids or salts thereof or anthracene mono- or di-sulphonic acids or salts thereof. Sulphonic acids or their salts are mixed with water or oil to form the treating bath and the oils generally used are linseed oil, cotton seed oil and other fatty substances.

Quenching compositions of the above types are defective in a number of respects among which are that water quenching causes stress and strain in the steel which tend to warp and crack the steel. Oil quenching is expensive because the oil deteriorates rapidly in use and must be refined, fortified or be continuously replaced with fresh oil.

It has now been discovered that an excellent thermally stable quenching composition for metals such as steel and steel alloys can be provided which comprises a mineral oil base containing a critical amount within the range of from about 1.75% to about 3.0% by weight and preferably between 2.0% and 3.0% of an artificial resin prepared by polymerizing cycloalkene hydrocarbons or lower polymers thereof with linolenic acid oils and their derivatives.

The cycloalkene hydrocarbons of which preferred are the cycloalkadiene hydrocarbons such as cyclopentadiene hydrocarbons, can be obtained by cracking of petroleum hydrocarbons, from domestic gas production or from coal tar industry. Cycloalkene hydrocarbons include cyclopentadiene, dicyclopentadiene, lower polycyclopentadienes, methyl cyclopentadiene and the like.

The linolenic acid oils and derivatives thereof which are used in the copolymeric resin include products having an iodine value of around 100—150 and containing at least 35% linolenic acid (diene) not more than 10% linolenic acid (triene) and not more than 25% saturated fatty acids. Such oils can be exemplified by soybean oil, perilla oil, cottonseed oil, hempseed oil, sunflower oil, walnut oil, poppyseed oil, sesame oil, maize oil, their acids and mixtures thereof.

The reaction can be conducted with or without the use

2

of a catalyst. The catalysts include salts of heavy metals such as nickel naphthenate or halides of amphoteric metals such as tin tetrachloride or bromide or iodide, or chlorides of antimony, bismuth and aluminum, as well as boron fluoride and dihydroxy fluoboric acid.

The temperature of the reactions can vary from about 50° C. to above 300° C. The reaction time varies depending upon the reactants, temperature, oil-solubility, and viscosity or physical state of the final product. In general, the reaction time varies from 2 to 24 hours.

The copolymer can be modified by introducing into the copolymer small amounts of various terpenic materials such as cyclic terpenes including dipentene, terpenolene, limonene, camphene, bornylene, or turpentine and pine oil and derivatives thereof.

The amounts of cycloalkene hydrocarbons and linolenic acid oils and derivatives thereof used to form the polymer can be varied from 5% to 95% and from 95% to 5%, respectively. If terpenic materials are introduced into the reaction mixtures, they are present in amounts of from 5% to 20%, based on the cycloalkene hydrocarbon.

Copolymers of this type can be prepared by the method described in the Journal of the American Oil Chemist's Society, volume 3 November 1954, page 543. Examples of such copolymers include copolymers of cyclopentadiene with soybean oil, or perilla oil, or poppyseed oil, or copolymers of dicyclopentadiene with soybean oil or mixtures of soybean oil and dipentene. A particularly preferred copolymer is sold commercially by Spencer Kellogg and Sons under the trade name "Cykelsoy" being a dicyclopentadiene soybean oil condensation product polymerized by heating at around 585—90° F. and having the following properties:

|    |                           |        |
|----|---------------------------|--------|
| 35 | Viscosity (Gardner-Holdt) | Z2     |
|    | Acid number               | 6.2    |
|    | Color (Gardner)           | 11     |
|    | Specific gravity          | 0.9705 |
| 30 | Saponification number     | 168.3  |
| 40 | Iodine number             | 129.7  |

Other examples of resinous additives used in quenching compositions of this invention are prepared as follows:

*Example I.*—About equal amounts of cyclopentadiene and soybean oil were reacted at about 250° C. in the presence of dihydroxyfluoboric acid catalyst for about 3 hours. The polymer was oil soluble.

*Example II.*—The procedure of Example I was followed using perilla oil instead of soybean oil.

*Example III.*—The procedure of Example I was followed using poppyseed oil instead of soybean oil.

Other suitable resins prepared by the method described above include copolymers of dicyclopentadiene/cottonseed oil, terpolymer of dicyclopentadiene/soybean/perilla oils and methylcyclopentadiene/soybean oil copolymer.

Minor amounts of from about 0.1 to 2% of secondary additives can be used in compositions of this invention. Particularly preferred are dispersants which can be of the ash-forming and/or ashless type dispersants such as metal sulfonates or phenates or ashless polymeric dispersants. The sulfonates and phenates include alkali and alkaline earth metal (Na, Ca, Ba) petroleum sulfonate, waxbenzene sulfonate, alkyl naphthalene sulfonate, alkyl phenate, dibutyl phenol sulfide, octylphenol-formaldehyde condensation product and the like. The ashless dispersants include oil-soluble nitrogen-containing polymeric dispersants such as Du Pont's PL-164A, LOA564, and LOA565 which are described in U. S. Pat-

ents 2,660,044, and 2,734,496 or Rohm and Haas's ashless dispersant "Acryloid 966" described in Petroleum Engineer, May 1956, page C-32. Other specific alkyl methacrylate ashless dispersants are vinyl pyridine/alkyl methacrylate polymers, vinyl pyrrolidone/alkyl methacrylate polymers such as 2-methyl-5-vinyl pyridine/mixed lauryl and octadecyl methacrylates, vinyl pyrrolidone/lauryl methacrylate copolymers and the like.

The oils which comprise the major proportion of the quenching compositions are mineral oils obtained as distillates from various types of crude oil such as paraffinic, asphaltic or mixed base crudes. The oils should have a flash point of above 300° F. and a Saybolt Universal viscosity at 100° F. of above 80 seconds and preferably from about 100 to about 200 seconds. Blends of different petroleum oils or mixtures of petroleum and fixed oils such as palm, rapeseed, and castor oils can be used.

The following compositions illustrate the invention:

|                                                                        | Percent |
|------------------------------------------------------------------------|---------|
| Composition A:                                                         |         |
| "Cykelsoy" <sup>1</sup>                                                | 2       |
| Mineral oil (100 SUS, 100° F.)                                         | 98      |
| Composition B:                                                         |         |
| "Cykelsoy" <sup>1</sup>                                                | 3       |
| Mineral oil (100 SUS, 100° F.)                                         | 97      |
| Composition C:                                                         |         |
| "Cykelsoy" <sup>1</sup>                                                | 2       |
| Ca petroleum sulfonate oil-soluble                                     | 1       |
| Mineral oil (100 SUS, 100° F.)                                         | 97      |
| Composition D:                                                         |         |
| "Cykelsoy" <sup>1</sup>                                                | 2       |
| Lauryl methacrylate-diethylaminoethyl methacrylate copolymer (PL-164A) | 1       |
| Mineral oil (100 SUS, 100° F.)                                         | 97      |
| Composition E:                                                         |         |
| "Cykelsoy" <sup>1</sup>                                                | 2       |
| Ca salt of octyl phenol-formaldehyde condensation product              | 1       |
| Mineral oil (100 SUS, 100° F.)                                         | 97      |

<sup>1</sup> "Cykelsoy"—Spencer Kellogg and Sons Product, as defined in column 2, lines 28 to 40.

Hardening metals such as steel by quenching operation can be done by any suitable means well known in the art. In essence the method of hardening steel by quenching comprises heating the metal to a temperature above its critical temperature and thereafter quenching the metal by immersion in a quenching oil composition of the present invention. The meaning of hardening steel by quenching is well understood in the art as evidenced by reference to Lubrication for September 1951, or Forbes text on "Lubrication of Industrial and Marine Machinery" (second edition), chapter 31.

The effectiveness of compositions of this invention as quenching media is demonstrated by the data presented in Table I in which the test compositions were subjected to the 5-second quench test, the hot-wire quench test and the beaker oxidation test. The 5-second quench test is described in Petroleum, January 1945, page 17.

The hot-wire quench test is a measure of the maximum amount of energy which a hot wire will dissipate to an oil. The maximum amount of energy which a hot wire will dissipate to the oil may be determined by increasing the current through the wire continuously until burnout occurs. The maximum energy can then be calculated from voltage and current measurements:

$$\text{Energy (max)} = V \cdot I_{\text{max}} = P_{\text{max}} \times R$$

where  $I$  = current and  $R$  is the resistance of the wire.

The bright quench test rating is a measure of the amount of deposits formed on the surface of the metal test specimen after it has been quenched in an oil that has been previously aged at 250° F. The specimens are rated 1 for clean and 10 for dirty.

4  
Table I

| Composition                                                                                                                                     | 5-Second Quench Test Speed, Percent | Hot-Wire Quench Test Rating (I <sup>2</sup> max.) | Bright Quench Rating (1=clean, 10=very dirty), Days |   |   |    |
|-------------------------------------------------------------------------------------------------------------------------------------------------|-------------------------------------|---------------------------------------------------|-----------------------------------------------------|---|---|----|
|                                                                                                                                                 |                                     |                                                   | 1                                                   | 3 | 5 | 7  |
| Mineral oil (100 SUS 100° F.)                                                                                                                   | 15                                  | 320                                               | 10                                                  | 3 | 4 | 5  |
| Composition A                                                                                                                                   | 29                                  | 720                                               | 3                                                   | 3 | 3 | 4  |
| Composition B                                                                                                                                   | 29                                  | 710                                               | 3                                                   | 3 | 3 | 4  |
| Composition U (mineral oil +4% "Acryloid 710")                                                                                                  |                                     | 410                                               | 10                                                  |   |   | 10 |
| Composition V (mineral oil +6% Santodex <sup>2</sup> )                                                                                          |                                     | 380                                               | 10                                                  |   |   |    |
| Composition W (mineral oil +1.0% Cykelsoy)                                                                                                      |                                     | 392                                               |                                                     |   |   |    |
| Composition X (mineral oil +1.5% Cykelsoy)                                                                                                      |                                     | 449                                               |                                                     |   |   |    |
| Composition Y (mineral oil +4.0% Cykelsoy)                                                                                                      |                                     | 671                                               |                                                     |   |   |    |
| Composition Z (mineral oil +5% copolymer of cyclopentadiene and a vegetable oil having an iodine number above 150 and above 35% linolenic acid) |                                     |                                                   |                                                     |   |   | 10 |

<sup>1</sup> Acryloid 710=polymerization product of esters of methacrylic acid and higher fatty alcohols described in U. S. Patent 2,712,726.

<sup>2</sup> Santodex=copolymers of C<sub>2</sub>-C<sub>12</sub> olefin and styrene.

Compositions C, D and E of this invention when tested as described above give substantially the same results as obtained with Compositions A and B.

I claim as my invention:

1. A quenching oil composition consisting essentially of a major amount of a mineral oil having a viscosity of from 100 to 200 SUS at 100° F. containing from about 1.75% to about 3.0% of an oil-soluble copolymer obtained by reacting a cycloalkadiene hydrocarbon and a linolenic acid oil having an iodine value between 100 and 150 for 2-24 hours at a temperature of from 50° C. to 300° C.

2. The composition of claim 1, wherein the cycloalkadiene hydrocarbon is cyclopentadiene.

3. The composition of claim 1, wherein the cycloalkadiene hydrocarbon is dicyclopentadiene.

4. A quenching oil composition consisting essentially of a major amount of mineral oil having a viscosity of about 100 SUS at 100° F. containing from about 2% to about 3% of an oil-soluble copolymer obtained by reacting dicyclopentadiene and soybean oil for about 3 hours at about 250° C. until the viscosity of the copolymer is about Z2 (Gardner-Holdt), and from about 0.1%

5. A quenching oil composition consisting essentially of a major amount of mineral oil having a viscosity of about 100 SUS at 100° F. containing from about 2% to about 3% of an oil-soluble copolymer obtained by reacting dicyclopentadiene and soybean oil for about 3 hours at about 250° C. until the viscosity of the copolymer is about Z2 (Gardner-Holdt), and from about 0.1% to 2% of a dispersant selected from the group consisting of oil-soluble metal sulfonate, metal phenate and oil-soluble nitrogen-containing polymeric compound.

6. The composition of claim 5, wherein the dispersant is an oil-soluble calcium petroleum sulfonate.

7. The composition of claim 5, wherein the dispersant is lauryl methacrylatediethylamino ethyl methacrylate copolymer.

8. A method of hardening steel comprising heating such steel to a temperature above its critical temperature and thereafter quenching such steel by immersion in the quenching oil composition of claim 1.

9. A method of hardening steel comprising heating such steel to a temperature above its critical temperature and thereafter quenching such steel by immersion in the quenching oil composition of claim 4.

10. A method of hardening steel comprising heating such steel to a temperature above its critical temperature and thereafter quenching such steel by immersion in the quenching oil composition of claim 5.

(References on following page)

## References Cited in the file of this patent

## UNITED STATES PATENTS

|           |          |               |             |
|-----------|----------|---------------|-------------|
| 2,340,724 | Horst    | Feb. 1, 1944  | 2,536,403   |
| 2,387,895 | Gerhardt | Oct. 30, 1945 | 2,573,940   |
| 2,485,103 | Mapes    | Oct. 18, 1949 | 2,710,842   |
|           |          |               | 5 2,734,031 |
|           |          |               | 2,799,606   |

|                |       |               |
|----------------|-------|---------------|
| Wallace et al. | ----- | Jan. 2, 1951  |
| Von Fuchs      | ----- | Nov. 6, 1951  |
| Heisig et al.  | ----- | Jan. 14, 1955 |
| McNaughtan     | ----- | Feb. 7, 1956  |
| Freeman        | ----- | July 16, 1957 |